

May 21, 1929.

J. W. SMITH

1,714,144

METHOD OF MAKING METAL WHEELS

Filed April 3, 1923

2 Sheets-Sheet 1

FIG. I.



FIG. II.



FIG. III.



WITNESSES:

*John C. Bergeron*  
*Alfred E. Ischinger*

INVENTOR:

*John W. Smith,*  
BY *Fralley & Paul*  
ATTORNEYS.

May 21, 1929.

J. W. SMITH

1,714,144

METHOD OF MAKING METAL WHEELS

Filed April 3, 1923

2 Sheets-Sheet 2



FIG. IV



FIG. V



WITNESSES:

*John C. Beymer*  
*Alfred E. Dachinger.*

INVENTOR:

*John W. Smith,*  
BY *Fralley, Paul*  
ATTORNEYS.

## UNITED STATES PATENT OFFICE.

JOHN W. SMITH, OF PHILADELPHIA, PENNSYLVANIA.

## METHOD OF MAKING METAL WHEELS.

Application filed April 3, 1923. Serial No. 629,585.

This invention relates to the manufacture of metal wheels having a tapering cross-section decreasing in thickness from the central portion to the peripheral edge thereof. Heretofore wheels of the type referred to have embodied two or more rigidly connected parts; that is to say, more specifically, a disk portion proper with an attached hub, and the fundamental object of my present invention is to provide a one piece composite disk and hub. In other words the primary object attained by my invention is a unitary hub and disk.

Incident to the production of an integral hub and disk in accordance with my novel method there will be a corresponding decrease in the weight and amount of material involved as compared with articles of a like character manufactured according to prevailing practice, and said economical phases are likewise important objects resultant from my present invention.

Other objects are to produce a metal disk having an evenly distributed thickness through its area no matter whether or not the cross-section be tapered or an even gage; to ensure a finished article devoid of any tendency to distortion; and to avoid any waste of stock during the process of manufacture.

With the foregoing and other objects in view, my invention consists essentially in the novel method and manner of making a unitary disk and hub from a drop forged blank, and adjunctively the said unitary article produced thereby, as hereinafter fully set forth.

In the further disclosure of the invention reference is to be had to the accompanying drawings constituting a part of this specification, and in which like designating characters distinguish the same or corresponding parts in all the views.

Figure I is a plan view of a convenient form of drop forged blank from which my novel type of disk is produced.

Figure II is a section on the line II-II in the preceding figure.

Figure III is a sectional view illustrative of the initial step or transformation of the drop forged blank into disk formation.

Figure IV is a similar view showing the second step or transformation of the disk proper into tapered cross-section; and

Figure V is a like view illustrative of the third step, or the formation of the disk web into conical cross-section.

In carrying out my invention and having reference more in detail to the drawings I employ a circular blank or drop forging 6 conveniently—though not essentially—of the cross-section shown by Figures I and II; 60 which is, to be more specific, the drop forging 6 is formed with co-axial cupped bosses 7, 8 that constitute, as hereafter set forth, the hub of the finished article, and a web portion 9. This blank or drop forging 6 is of approximately one-half the required finished diameter and five times the average finished gage or thickness. The drop forging or blank 6 is heated to the necessary degree and placed upon a suitable supporting element or turn-table 10, Figure III, of an appropriate mill—not shown—and subjected to an expanding operation, by means of one or more forging rollers 11. The forging roller or rollers 11 is, or are, adapted for radial outward movement relative to the axis of the drop forging or blank 6, thereby producing a reduced gage or thickness of metal throughout the disk web 9. This roll or rollers 11 is or are, it will be observed, generally conical in form except 80 for a tread portion 12 that is rounded at 13 so as to assist the gradual displacement of the metal from the central portion of the blank or forging 6 towards the periphery thereof, and incidentally obviating any tendency to fracture which might otherwise result. In practice, I prefer to employ two forging rollers 11 in opposed radial relation relative to the axis of the forging or blank 6, and arrange them to travel outwards with a uniform rate 85 of speed. Also, it is worthy of note, at this juncture, that I prefer to use what is commonly known as a three pass rolling mill feeding the rollers 11 across the disk web 9 thrice at a very rapid speed, approximately 90 of five seconds' duration for each pass. In the drawings the formation assumed by the disk web 9 after the first pass is clearly shown by Figure III. Obviously the aforesaid cupped bosses 7, 8 are made from comparatively thick 95 blanks and consequently well adapted for drop forging, as will be readily understood by those conversant with the art.

It is to be remarked that I accomplish the foregoing disk forming steps with one heat 105 of the drop forging or blank 6, thereby effecting an economy in time and labor. The wheel produced as just described is now ready to be flanged and formed to the required finished shape in a suitable drawing press, while 110

the machining of the cupped bosses 7, 8 is later carried out as will be clearly understood by those conversant with the art to which this invention appertains.

5. At the beginning of each pass the forging rollers 11 are forced into the blank reducing it to a predetermined thickness by traveling in a straight line in a radial direction; while the turntables 10 and 14 may have a parallel 10 zone at the outer periphery with respect to said straight line path of the rollers, and a tapered zone near the hub as illustrated in Figures III, IV and V, thereby rolling a disk of tapered cross-section at the hub zone, 15 and an even gage at the outer periphery. Heretofore the use of thin metal disks of varied cross-section, or tapered section, was limited to restricted methods of producing same, but I have discovered that by a combination 20 spinning and rolling process I am enabled to produce the integral hub and disk type of wheel herein described. Thus it will be easily seen from Figure IV that the roller face 12 rolls the metal to the required thickness by cooperation with the turntable 10, 25 while the face 11 and round corner 13 function as a spinning portion to stretch the dished portion of the blank in advance of the rolling action. Figure III shows the up- 30 turned edge 9' of the disk 9, which flares up very high during some of the passes when the rollers are about two-thirds out from the center; and, obviously, said flared up edge must be acted upon by a spinning operation since 35 it is not virtually in contact with turntable 10.

In most instances wheels of the type referred to are required to have a fine finish and a greater or lesser degree of concavo-convexity so as to ensure greater rigidity and in this 40 connection I immerse the wheel formed as before set forth in a suitable diluted acid solution to remove all scale or other matter from the surface thereof and then subject the same to a cold rolling process. This cold 45 rolling process may conveniently be carried out by placing the wheel on to a conical supporting element or turn table 14—Figure V—having an associated forging roller or rollers 15 of the character above described. This 50 cold rolling operation results in the transformation of the disk web 9 from the dotted line position indicated in Figure V to the full line section showing, whereby said disk is rendered much stiffer at the hub portion than 55 if so shaped by direct pressure. Or, the formation of the blank 6 to more or less conical cross-section may be effected by hot-rolling 60 as in the case of relatively heavy vehicle wheels.

60. From the foregoing description it will be obvious that any desired cross-sectional configuration of the disk may be obtained by varying the profile of the element or turn table 10, but I desire to particularly emphasize 65 the fundamental object of my invention

which is the production of a wheel having an integral hub and disk by the method hereinbefore described.

By the use of my improved method of manufacture, wheels of the type referred to can 70 be produced at a greatly reduced cost and corresponding economy in stock utilized, with a considerable saving of time and labor.

Having thus described my invention, I 75 claim:

1. The method of making wheels which consists in drop forging a blank to provide a hub and integral surrounding concentric web portion, expanding said web radially outward from the hub portion by a combined 80 rolling and spinning operation to diminish the gage, stretching the peripheral remainder to uniform thickness by spinning, and finally cold-rolling said expanded web to the required shape. 85

2. The method of making wheels which consists in drop forging a blank to provide opposed axially concentric hub portions with an integral surrounding web, expanding said web radially outward to a definite zone thickness for a predetermined distance from the hub portions by a combined rolling and spinning operation, and subsequently expanding the web when cold to dished cross-section by a similar operation. 90

3. The method of making wheels which consists in drop forging a blank to provide an enlarged central portion with an integral surrounding web, expanding the web of said blank while hot radially outward for a limited distance by a combined rolling and spinning operation to gradually diminish its gage, shaping said expanded web when cold to conically dished cross-section by a similar operation, and finally machining the enlarged center portion to form a finished hub. 100

4. The method of making wheels which consists in drop forging a blank to provide concentric bosses with an integral surrounding web, expanding said web radially outward from the bosses for a predetermined distance by a combined rolling and spinning operation with one heat, cold rolling said expanded blank by a similar operation to secure a finished surface and to shape said 110 expanded web to required form, and finally machining the bossed portion to provide a finished hub.

5. The method of making wheels which consists in drop forging a comparatively 120 thick blank to provide axially opposed bossings with an intermediate integral web, expanding said web while hot radially outward from the bossings for a limited distance by a combined rolling and spinning operation to diminish the gage, cold rolling the expanded web on a suitable form to conical cross-section and required shape by a corresponding operation, and finally machining the hub. 125

6. As an article of manufacture a metal 130

disk wheel having an integral hub and conically dished web portion gradually diminishing in thickness outwardly from the hub zone for a predetermined distance with a uniform thickness at the outer peripheral portion.

7. As an article of manufacture a blank for disk wheels having an integral hub and a conically dished web portion of outward and gradually diminishing thickness merging into a zone of uniform gage with a reinforced outer peripheral rim.

8. The art of producing a disk wheel for automotive use which consists in progressively expanding an annular zone of a suitably shaped heated blank by a composite rolling and spinning operation, and subsequently shaping such expanded portion when cold incidental to a corresponding operation. 15

In testimony whereof, I have hereunto signed my name at Philadelphia, Pennsylvania, this 27th day of March, 1923.

JOHN W. SMITH.